

## UNITED STATES PATENT OFFICE

1,930,133

## DECOLORIZING PROCESS

Marvin J. Reid, Rochester, N. Y., assignor to  
 Eastman Kodak Company, Rochester, N. Y.,  
 a corporation of New York

No Drawing. Application June 14, 1932  
 Serial No. 617,257

5 Claims. (Cl. 252—1)

This invention relates to a process of decolorizing cellulose ester materials, and more particularly to a process for decolorizing dyed cellulose acetate sheets or films.

5 A variety of cellulose ester plastic products, especially photographic films, thin sheeting used for wrapping purposes and the like, are colored by the incorporation of dye-stuffs into the dopes from which they are produced or by direct dye-  
 10 ing of the sheet. In the course of manufacture and use of such products, a considerable amount of waste is produced which, if not recovered, represents a serious economic loss to the manufacturer or consumer. In the interest of econ-  
 15 omy it has become necessary to treat such materials and recover the valuable ingredients which they contain. One of the difficulties en-  
 countered in such recovery processes is the removal of dyestuffs and other coloring matter.  
 20 Although colored films and sheetings may be bleached by various solvents and solvent combi-  
 nations, and the dye eventually removed, such processes are sometimes ineffective to completely decolorize the material and, unless the material  
 25 is reduced to an extremely fine state of subdivi-  
 sion, are generally exceedingly time-consum-  
 ing and inconvenient. In the case of nitrocel-  
 30 lulose film scrap, there is considerable danger in grinding the material sufficiently fine for penetration of the bleaching solvents due to the inflammable character of nitrocellulose.

The present invention has for its principal object to provide a simple and effective method of decolorizing cellulose ester scrap materials, such as those produced from dyed photographic film and thin sheeting. A further object is to provide a method in which the decolorizing or bleaching agent may act upon the material with a minimum consumption of time. Another ob-  
 40 ject is to provide a method whereby cellulose films produced from such materials as cellulose nitrate, cellulose acetate, or other cellulose organic esters, or cellulose ethers, may be de-  
 45 colorized without preliminary subdividing and grinding operations. A specific object is to pro-  
 vide a method for decolorizing a dyed cellulose acetate sheeting scrap with the customary bleaching agents. Other objects will herein-  
 after appear.

50 These objects are accomplished by the follow-  
 ing invention which, in its broadest aspects, comprises a combination of the following steps. The colored scrap material is first dissolved in a suitable solvent to produce a colored solu-  
 55 tion or dope. This is mixed with a suitable

precipitant, such as water, or other non-solvent, the cellulosic material being thereby precipitated in a light, porous form still having most of the dye incorporated therewith. The precipitated material is filtered off, bleached by mixing with 60 a suitable bleaching agent such as chlorine water and thereafter leached counter-currently with methyl alcohol which removes the soluble chlo-  
 65 rides produced in the bleaching operation. The decolorized material is washed, dried, and is 65 then in a condition immediately available for re-use in the manufacture of films, cellulosic sheeting and allied products.

In the following example, I have set forth one of the preferred embodiments of my invention, 70 but it is included merely for purposes of illus-  
 tration and not as a limitation thereof.

## Example

10 grams of colored cellulose acetate thin 75 sheeting scrap material is dissolved in 100 grams of acetone to produce a colored dope. The dope is then run into an excess of hot water contained in a suitable receptacle and maintained at a temperature of 120° F. The soft, porous 80 cellulose acetate is immediately precipitated still containing the dye-stuff. After precipitation is completed, the material is filtered from the solution and bleached with saturated chlorine water for one hour at room temperature, which 85 converts the dyestuffs to colorless compounds and occasions the formation of soluble chlorides. It is then separated from the bleaching solu-  
 90 tion and leached by three one-hour counter-  
 current changes of methyl alcohol at a tem-  
 perature of 80° F. to remove the soluble chlo-  
 95 rides formed during the chlorine water treat-  
 ment. The leached precipitate which is light and porous in character is then dried after which it may be re-used in the manufacture of 95 photographic film, thin sheeting and the like.

Although in the above example I have de-  
 scribed my process with reference to colored cellulose acetate thin sheeting, it is not in any way limited thereto. The process is equally ap-  
 100 plicable to the treatment of thin or thick sheets of cellulosic materials, although it is desirable in the case of thicker sheeting to cut the ma-  
 terial into smaller pieces than is necessary with thinner stock. The invention is, of course, not 105 limited to the treatment of cellulose acetate, but may be applied to the decolorizing of cellulose nitrate, cellulose ethers, such as benzyl cellulose, and the higher or mixed cellulose organic esters, such as cellulose propionate, cellulose 110

butyrate, or cellulose acetate propionate, cellulose acetate butyrate, and the like.

The cellulosic material will in the first instance be dissolved in any appropriate solvent. Solvents for cellulose acetate, for example, include acetone, methylene chloride, methyl acetone, methyl acetate, ethyl acetate, 1-4 dioxane, ethyl lactate, diacetone alcohol, and others. Likewise, the precipitant may be selected from a wide range of suitable substances, typical examples of which for cellulose acetate include water, methyl alcohol, ethyl alcohol, and dilute aqueous acetic acid of approximately 20% strength. Other suitable cellulose acetate precipitants are disclosed in the copending application of C. J. Malm and C. R. Fordyce, Serial No. 553,646, filed July 28, 1931, relating to the use of ethers as precipitants. The solvents and precipitants of themselves form no part of the present invention, since they are for the most part well known to those skilled in the art, both solvents and precipitants, of course, being selected upon the basis of suitability for use with the particular cellulosic compound dealt with.

Although I have found chlorine water to be a particularly effective bleaching agent for removing the color from the precipitated cellulosic material, I may use with equally satisfactory results sodium and calcium hydrochlorites, chlorine gas, and other known bleaching agents.

My process is particularly distinguished by the fact that cellulose acetate or other cellulosic material are brought into a physical condition in which the bleaching agent can quickly and effectively penetrate therein and perform its decolorizing function. This makes possible a pronounced saving in the recovery of colored scrap sheeting and photographic film, inasmuch as the material is immediately brought into a condition in which the dye may be removed directly, thereby eliminating the necessity for the dangerous and inconvenient grinding operations of the prior art. So far as I am aware, no process thus far known to the art involves a method whereby the cellulosic material is brought into a porous, precipitated condition prior to the bleaching treatment.

In the above specification and appended

claims, reference to cellulosic scrap material is intended to include scrap produced from either photographic film or from thin sheeting, such as that used for wrapping purposes, or any other cellulosic scrap material.

As many apparently widely different embodiments of this invention may be made without departing from the spirit thereof, it is to be understood that I do not limit myself to the foregoing example or description except as indicated in the following patent claims.

What I claim as my invention and desire to be secured by Letters Patent of the United States is:

1. The process of decolorizing a dyed cellulosic scrap material which comprises dissolving the material in a solvent therefor, precipitating the material from solution by means of a non-solvent therefor, and thereafter bleaching the dye out of the precipitate while in a relatively open, porous condition.

2. The process of decolorizing a dyed cellulosic scrap material which comprises dissolving the material in a solvent therefor, precipitating the material from solution by means of water, and thereafter bleaching the dye out of the precipitate while in a relatively open, porous condition.

3. The process of decolorizing a dyed cellulose ester scrap material which comprises dissolving the material in a cellulose ester solvent, precipitating the cellulose ester from solution by mixing with a cellulose ester non-solvent therefor, and thereafter treating the precipitate while in a relatively open, porous condition with a bleaching agent.

4. The process of decolorizing a dyed cellulose acetate sheet scrap material which comprises dissolving the material in acetone, passing the resulting solution into an excess of water, and thereafter treating the dyed cellulose acetate precipitate while in a relatively open, porous condition with an aqueous chlorine-containing bleaching agent.

5. The process of decolorizing a dyed cellulose acetate sheet scrap material which comprises dissolving the material in acetone, passing the resulting solution into an excess of water, and thereafter treating the dyed cellulose acetate precipitate while in a relatively open, porous condition with chlorine water.

MARVIN J. REID.